

# United States Patent

[11] 3,617,191

[72] Inventor **William Wade Caldwell**  
Abbeville, S.C.  
[21] Appl. No. **761,796**  
[22] Filed **Sept. 23, 1968**  
[45] Patented **Nov. 2, 1971**  
[73] Assignee **Deering Milliken Research Corporation**  
**Spartanburg, S.C.**

[54] **TREATMENT OF TEXTILE MATERIAL WITH  
BORIC ACID**  
**11 Claims, No Drawings**

[52] U.S. Cl. .... **8/115.7,**  
                      **8/115.5, 8/116, 8/116.2**  
[51] Int. Cl. .... **D06m 9/00**  
[50] Field of Search. .... **8/115.5,**  
                      **115.7**

[56] **References Cited**  
UNITED STATES PATENTS  
3,475,114 10/1969 Bolinger et al..... 8/127.5  
3,467,487 9/1969 Kirschnek ..... 8/115.5  
3,471,466 10/1969 Hayes..... 260/21

*Primary Examiner—George F. Lesmes  
Assistant Examiner—B. Bettis  
Attorneys—Norman C. Armitage and H. William Petry*

**ABSTRACT:** A process for improving the resistance to discoloration during irradiation of a blended textile material of polyamide and cellulosic fibers which comprises applying to said textile material a metal salt or an amino salt catalyst, boric acid and a monomer containing ethylenic unsaturation and a group capable of reacting with hydroxyl groups and irradiating the treated textile material to polymerize said monomer.

## TREATMENT OF TEXTILE MATERIAL WITH BORIC ACID

One of the important processes for treating textile material to achieve minimum care properties, that is, wash and wear or durable press characteristics, involves the application of a polymerizable material to the textile material and the irradiation thereof to graft polymerize the monomer. Subsequently, the textile material is cured generally either in fabric or garment form to provide the minimum care properties.

It has been found in such processing of textile material that the irradiation step may cause a change in the color of the textile material. With certain dyed fabrics, there is a tendency for the fabric color to change and with white or undyed fabrics there is a tendency toward yellowing. This condition has limited the available color selections and has increased the quantity of off-quality goods.

In accordance with the present invention, a novel process has been discovered for minimizing the color change of textile material during irradiation. The process of the invention comprises applying a vinyl monomer having dual functionality and boric acid to a textile material and irradiating the treated textile material without causing a significant change in the color thereof. Preferably, the proportion of boric acid based on the dry weight of textile material is between about 0.5 percent and 3 percent and particularly between about 1 percent and 2 percent.

The textile material treated in accordance with the present invention may include any of the conventional natural and synthetic fibers. Advantageously, the textile material includes polyamide fibers in a blend with natural or synthetic fibers and particularly a blend with viscose rayon or cotton fibers.

The process of the present invention is particularly useful with polyamide textile material which has been dyed with conventional polyamide acid or dispersed dyestuffs. The color change commonly encountered heretofore was particularly observable with red dyestuffs which tended to lose their color. However, in accordance with the process of the present invention, as pointed out above, such a change is substantially eliminated.

The vinyl monomer with dual functionality employed in the process of the invention advantageously comprises between about 1 percent and 30 percent by weight of the textile material and preferably between about 5 percent and 15 percent. Suitable monomers include compounds containing the group  $\text{CHR}^4=\text{CR}^3$ , wherein  $\text{R}^3$  is selected from hydrogen and methyl and  $\text{R}^4$  is selected from hydrogen and lower alkyl (preferably, containing one to four carbon atoms). The preferred compounds for use in accordance with this invention contain this group, preferably as



in combination with one of the following reactive groups, 55 preferably adjacent thereto for increased reactivity of the unsaturated group.

Acid reactive groups are generally those found in the textile resins presently employed in the resin treatment of cellulosic fabrics, e.g., methylol, epoxy, acetal, alkylated methylol, aldehyde,



wherein  $\text{R}^6$  is hydrogen or alkyl,  $-\text{N}=\text{C}-\text{O}$ ,  $-\text{N}=\text{C}-\text{S}$  and the like. These groups are characterized by their ability to combine with the hydroxy groups of the cellulose molecule under textile resin curing conditions.

Typical compounds having both a polymerizable group and a group reactive with hydroxy groups of cellulose include those having the following formulae:



wherein  $\text{R}'$  is selected from hydrogen, lower alkyl, and the residue of an aldehyde;  $\text{R}^2$  is selected from hydrogen, lower alkyl, and  $-\text{CX}-\text{CR}^4=\text{CHR}^4$ ;  $\text{R}^3$  is selected from hydrogen and methyl;  $\text{R}^4$  is selected from hydrogen and lower alkyl; and  $\text{X}$  is selected from sulfur and oxygen.

Additional suitable compounds include imides, such as



and the like; vinyl sulfonamides, such as



and the like, wherein  $\text{R}^1$ ,  $\text{R}^2$ ,  $\text{R}^3$ ,  $\text{R}^4$  and  $\text{X}$  are as defined above. The



35 can have substituted therefor



40 and sulfonium if desired.

In any of the compounds shown herein, particularly those characterized by formula I above, the



45 groups may have substituted therefor



and sulfonium if desired.

Additional compounds include anhydrides, such as



60 55 Preferred compounds characterized above are acrylamide compounds such as the methylol acrylamides, e.g.,



(N-methylol-methacrylamide),





yarns, threads or fabrics, although the presensitizing embodiment of this invention is most advantageously conducted on fabrics. Such fabrics can be woven, nonwoven, knitted, as desired.

Garments made from these fabrics can be produced in the conventional manner with no additional steps required and may be folded and pressed on conventional equipment, for example, a Hoffman press. The pressing cycle utilized is standard in the industry and generally involves pressing of the garment for a short period of time, followed by a curing operation in an oven. Alternatively, the garment may be set in a desired configuration under hot dry conditions, such as by hot pressing without steaming, for example, at temperatures up to about 200° C. for as long as necessary to produce the desired results.

The following examples illustrate particular embodiments of the invention but are not intended to limit the scope of the invention. In the examples, parts and percentages are by weight.

#### EXAMPLE I

A red stretch fabric made from a blend of nylon and viscose rayon fibers (30%/70%) is padded with an aqueous mixture containing about 18% N-methylol acrylamide (60% solution), 5% magnesium chloride catalyst (50%  $MgCl_2 \cdot 6H_2O$ ), 4% Polycryl TF-25 (an acrylic emulsion hand builder), 0.2% nonionic wetting agents and 2% boric acid. The fabric with about 70% wet pickup is dried to about normal moisture regain by heating at about 185° F. and then irradiated with a 1 megarad dose by passing the fabric through irradiation equipment having an insulated core transformer manufactured by High Voltage Equipment Corporation of Burlington, Mass. The fabric is dried in an oven to about normal moisture regain.

A control fabric is made according to the above procedure except the boric acid is omitted from the pad bath and replaced with an equal amount of magnesium chloride catalyst.

Portions of each of the resulting fabrics are made into slacks and pressed on a hot head press with a cycle of 5 seconds steam, 5 seconds bake and 5 seconds vacuum. The slacks are cured in an oven at a temperature of about 320° F. for about 10 minutes. Examination of the finished slacks shows that the slacks treated with the bath containing boric acid have a color substantially the same as the starting fabric while the slacks made with the control fabric have changed shade considerably.

#### EXAMPLE II

The procedure of this example is the same as that of example I except that the fabric is an olive color and the irradiation dose is reduced to 0.5 megarad. Examination of the slacks shows that the slacks produced according to the invention have a true olive color whereas the slacks made with the control fabric are brown in appearance.

#### EXAMPLE III

The procedure of this example is the same as that of example I except the irradiation dose is increased to two megarads.

The slacks made according to the process of the invention show the same superiority over the control fabric as observed in example I.

#### EXAMPLE IV

10 The procedure of this example is the same as that of example I except an undyed fabric is employed and the fabric is cured in fabric form. The fabric treated in accordance with the invention is without significant yellowing while the control fabric is visibly yellowed.

15 The above description and examples show that the present invention provides a novel process for minimizing the color change of dyed textile material or yellowing of white or undyed textile material. Furthermore, the invention is especially suitable for the treatment of textile material including polyamide fibers which has been dyed particularly with a red dyestuff.

20 It will be apparent from the above that various modifications in the formulations and procedures described in detail may be made within the scope of the invention. Therefore, it is intended that the invention be limited only by the following claims.

That which is claimed is:

1. A process for improving the resistance to discoloration during irradiation of a blended textile material of polyamide and cellulosic fibers which comprises applying to said textile material a metal salt or an amino salt catalyst, boric acid and a monomer containing ethylenic unsaturation and a group capable of reacting with hydroxyl groups and irradiating the treated textile material to polymerize said monomer.

30 2. A process according to claim 1 wherein between about 0.5% and 3% boric acid based on the dry weight of textile material is applied.

35 3. A process according to claim 1 wherein the treated textile material is irradiated with a dose between about 0.1 and 10 megarads.

40 4. A process according to claim 1 wherein between about 1% and 30% vinyl monomer based on the dry weight of textile material is employed.

45 5. A process according to claim 1 wherein the catalyst is selected from the group consisting of zinc nitrate and magnesium chloride.

6. A process according to claim 1 wherein the vinyl monomer is an acrylamide compound.

7. A process according to claim 6 wherein the acrylamide compound is N-methylol acrylamide.

8. A process according to claim 1 wherein the textile material has been dyed with a red dyestuff.

9. A process according to claim 1 wherein the vinyl monomer is an acrylamide compound, a catalyst is applied to the textile material and between about 1% and 2% boric acid based on the dry weight of the textile material is applied.

10. A textile material prepared according to the process of claim 1.

11. A textile material including polyamide fibers prepared according to the process of claim 9.

\* \* \* \* \*